



US005989322A

# United States Patent [19]

Riggs, Jr.

[11] Patent Number: 5,989,322

[45] Date of Patent: \*Nov. 23, 1999

[54] **CORROSION INHIBITION METHOD AND INHIBITOR COMPOSITIONS**[75] Inventor: **Olen Lonnie Riggs, Jr.**, Yukon, Okla.[73] Assignee: **A.S. Incorporated**, Alameda, Calif.

[\*] Notice: This patent is subject to a terminal disclaimer.

[21] Appl. No.: **09/205,839**[22] Filed: **Dec. 3, 1998****Related U.S. Application Data**

[62] Continuation of application No. 08/837,716, Apr. 22, 1997, which is a continuation-in-part of application No. 08/232, 282, filed as application No. PCT/US92/09511, Nov. 5, 1992, Pat. No. 5,510,057, which is a continuation-in-part of application No. 07/788,530, Nov. 6, 1991, Pat. No. 5,202, 058

[60] Provisional application No. 60/015,914, Apr. 22, 1996.

[51] **Int. Cl.<sup>6</sup>** ..... **C23F 11/10**[52] **U.S. Cl.** ..... **106/14.44; 106/14.14;**  
252/389.1; 252/396; 422/19[58] **Field of Search** ..... 106/14.44, 14.14;  
252/389.1, 396; 422/19[56] **References Cited****U.S. PATENT DOCUMENTS**

|           |         |                 |       |           |
|-----------|---------|-----------------|-------|-----------|
| 3,679,579 | 7/1972  | Preusser et al. | ..... | 585/808   |
| 3,776,835 | 12/1973 | Dvoracek        | ..... | 208/48 AA |
| 3,933,662 | 1/1976  | Lowe            | ..... | 252/387   |

|           |         |                 |       |           |
|-----------|---------|-----------------|-------|-----------|
| 4,124,512 | 11/1978 | Stournas et al. | ..... | 507/244   |
| 4,284,517 | 8/1981  | Chen et al.     | ..... |           |
| 4,440,625 | 4/1984  | Go et al.       | ..... | 208/48 AA |
| 4,619,756 | 10/1986 | Dickakian       | ..... | 208/48 AA |
| 4,866,969 | 9/1989  | Reismann et al. | ..... | 72/238    |
| 4,913,830 | 4/1990  | Lundberg et al. | ..... | 508/194   |
| 4,937,007 | 6/1990  | Damin et al.    | ..... | 507/90    |
| 5,104,518 | 4/1992  | Jager           | ..... | 208/125   |
| 5,139,643 | 8/1992  | Roling et al.   | ..... | 208/48 AA |
| 5,171,420 | 12/1992 | Forester        | ..... | 208/48 AA |
| 5,171,421 | 12/1992 | Forester        | ..... | 208/48 AA |
| 5,183,555 | 2/1993  | Forester        | ..... | 208/48 AA |
| 5,194,142 | 3/1993  | Forester        | ..... | 208/48 AA |
| 5,194,620 | 3/1993  | Roling et al.   | ..... | 548/112   |
| 5,202,058 | 4/1993  | Riggs, Jr.      | ..... | 252/387   |
| 5,211,834 | 5/1993  | Forester        | ..... | 208/48 AA |
| 5,211,835 | 5/1993  | Forester        | ..... | 208/48 AA |
| 5,292,425 | 3/1994  | Forester        | ..... | 208/48 AA |
| 5,342,505 | 8/1994  | Forester        | ..... | 208/48 AA |
| 5,510,057 | 4/1996  | Riggs           | ..... | 252/387   |

*Primary Examiner*—Anthony Green*Attorney, Agent, or Firm*—Harold D. Messner; Dehlinger & Associates[57] **ABSTRACT**

The present invention provides a method and compositions useful for inhibiting corrosion of a corrodible metal resulting from contact of water and air with the metal. In this method, a stannous salt and a hydrocarbyl substituted succinimide of a polyethylene polyamine, separately or in combination, are added to the water in a minor amount and reduce corrosion of the metal to a substantially low rate.

**4 Claims, No Drawings**

## CORROSION INHIBITION METHOD AND INHIBITOR COMPOSITIONS

This application is a continuation of pending U.S. application Ser. No. 08/837,716, filed Apr. 22, 1997, which is a continuation-in-part of provisional application No. 60/015,914, filed Apr. 22, 1996, and of application Ser. No. 08/232,282, filed May 6, 1994, now U.S. Pat. No. 5,510,057, which is the U.S. national stage of PCT/US92/09511, filed Nov. 5, 1992, which claims priority to U.S. application Ser. No. 07/788,530, filed Nov. 6, 1991, now U.S. Pat. No. 5,202,058.

### FIELD OF THE INVENTION

The present invention relates to a method for inhibiting corrosion of corrodible ferrous metal in a water-metal-air contact system by means of a dual corrosion agent system and compositions for the practice of the method.

### BACKGROUND OF THE INVENTION

Cooling water tower systems are usually fabricated of ferrous metal. A common problem is severe corrosion which results from water and air contact with the metal, especially in the case where the cooling water is brackish.

Chromate type inhibitors formerly used to reduce corrosion have been banned for use because of environmental impact problems. Consequently, there is a need for a new effective corrosion inhibitor system and, of course, for one which exhibits improved efficiency in inhibiting corrosion and which employs materials free of deleterious environmental impact. *Inhibitors currently available to the art, for example, phosphate, phosphonate, molybdate, nitrate and zinc types and the like, reduce carbon steel corrosion rates in brackish water to the amount on the order of 16 to 35 mils per year (mpy).* This is a serious rate and one hardly acceptable considering replacement and repair costs for cooling towers.

### SUMMARY OF THE INVENTION

The present invention provides a method and compositions useful for inhibiting corrosion of ferrous metal resulting from contact of water and air with the metal. In this method, a stannous salt and a hydrocarbyl substituted succinimide of a polyethylene polyamine are added to the water in minor amounts and cooperatively reduce corrosion of the metal to a substantially zero rate. While the amount of each agent for an effective inhibition is minor, in the range of about 0.1 to 100 ppm, a relatively concentrated solution is required for addition to the water. Suitable solvent media include the lower alkanols and mixtures thereof with or without added water. Isopropanol is preferred. The solvent component of the compositions varies depending on the particular imide and/or salt component employed and the concentration desired. In general, the lower alkanol portion of the medium is in the range from about 15 to 100 volume percent and the water portion is in the range from about 0 to 85 volume percent. A medium in the range from about 50 to 67 volume percent water is preferred. The relative amounts of the imide and stannous salt components desirably used vary depending upon the nature of the water in which the agents are employed. Satisfactory relative amounts by weight are in the range from about 0.5 to 10, preferably 0.8 to 2, and more preferably about 1 to 1 weight ratio.

### DETAILED DESCRIPTION OF THE INVENTION

The present invention is based upon novel corrosion inhibitor compositions and their cooperative use in a method

wherein corrosion of corrodible metals, e.g., low carbon, silica and mild steels and the like, is reduced to a negligible rate.

The corrosion inhibiting agents required for the practice of the present invention must disperse readily in water, especially brackish water. While the amount of each of the agents required for an effective inhibition is minor, e.g., in the range from about 0.1 to 100 ppm, preferably 0.5 to 10 ppm, a relatively concentrated solution is required before the solution is added to the water. Suitable solvent media include the lower alkanols, e.g., methanol, ethanol, propanol, isopropanol and mixtures thereof with or without added water. Isopropanol is preferred.

The solvent or medium component of the composition varies depending upon the particular imide and/or salt component employed and the concentration desired. In general, the lower alkanol portion of the medium is in the range from about 15 to 100 volume percent and the water portion is in the range from about 0 to 65 volume percent. A medium in the range from about 50 to 67 volume percent water is preferred.

The relative amounts of the imide and stannous salt components desirably used varies depending upon the condition of the industrial water in which the compositions of the invention are to be used. Satisfactory relative amounts by weight are in a range from about 0.5 to 10, preferably 0.8 to 2, and still more preferably about a 1 to 1 ratio.

In addition to a suitable medium for the agents and to enhance dispersion of the agents into water, the concentrates herein require an effective amount of a suitable wetting agent. An effective amount of a wetting agent is in the range from about 0.1 to 5, preferably 0.3 to 1, weight percent of the inhibitor agent. In general, the use of an amount of wetting agent in excess of about 5 weight percent is neither deleterious nor enhancing, but is, of course, not cost effective. Particular and preferred wetting agents for use in the compositions herein described are the polysorbate surfactants and mixtures thereof, preferably mono-9-octadecenoate poly(oxy-1,2-ethanediyl) groups. The sorbitol surfactants effectively disperse the inhibitors of the invention and also are believed to enhance corrosion prevention. Thus, in the absence of these surfactants, less effective corrosion inhibition is experienced, and where a non-sorbitol type surfactant has been used, markedly inferior corrosion inhibition has been experienced. The sorbitol surfactants used herein are known and prepared conventionally as known in the art, e.g., by the reaction of ethylene oxide with the mono-ester of 9-octadecenoic acid and sorbitol.

Stannous salts having an appreciable (at least 0.1 weight percent) solubility in water, in general, are suitable for use in the present invention. Representative stannous salts suitable for use include the chloride and its dihydrate, acetate, butyrate, octanoate, isobutyrate, hexadecanoate, and the like salts. The chlorides are a preferred group. Most preferred are the salts of organic mono-carboxylic acids having a carbon atom content in the range of from about 1 to 16, preferably 4 to 10 carbon atoms.

#### Example 1

A solution of stannous chloride was prepared by heating and stirring a mixture of ethanol and the dihydrate of stannous chloride to about 65° C. and then adding mono-5-octadecenoate poly (oxy-1,2-ethanediyl) sorbitol (about 20 ethanediyl groups) surfactant (1% by weight of the ethanol-stannous chloride mixture). Additional ethanol was added to obtain about a 20 weight percent solution of stannous chloride.

#### Succinimides

Succinimides of polyethylene polyamines are in general satisfactory for use in the invention. Preferred imides are

those obtained from substituted succinic acids or acid anhydrides known in the art in which the substituent is a hydrocarbyl group having a carbon atom content in the range of from 1 to about 15, more preferably an aliphatic hydrocarbon group, and most preferably an alkenyl group having a carbon atom content in the range of from 3 to about 15. Representative alkenyl groups include n- and iso-octenyl, pentenyl, dodecenyl and the like. These substituted succinic acids or anhydrides are known and are prepared by conventional reactions, e.g., by the free radical catalyzed addition of alpha-olefins to maleic acid and its anhydride.

The polyethylene polyamine component of these imides satisfactory for use in the invention contains from about 1 to about 8 ethylene groups and from 2 to about 9 amino groups. Representative polyamines include ethylene diamine, diethylene triamine, triethylene tetramine, tetraethylene pentamine, pentaethylene hexamine, mixtures thereof, unfractionated or crude preparative reaction product mixtures thereof and the like, and polyethylene polyamines. Tetraethylene pentamine is preferred. The polyamines are known and prepared by conventional reactions known in the art.

#### Example 2

N-octenyl succinimide of tetraethylene pentamine was prepared by placing one mole of the amine in a reaction flask fitted with an addition funnel containing one mole of n-octenyl succinic anhydride, a water collector, a stirring and heating means and a reflux condenser. While the amine was stirred, the anhydride in the funnel was slowly added to the flask. Upon completion of the addition, the resulting reaction mixture was heated to about 142° C., whereupon water of reaction started to distill over. At about 180° C., the resulting reaction product, viz., n-octenyl succinimide of tetraethylene pentamine, was a clear bright orange liquid. About one mole of water was collected in the collector, signifying that the imide-forming reaction was complete. The flask and its contents were then cooled to about 80° C., and sufficient isopropanol and distilled water were added to yield a solution which was 40 volume percent isopropanol, about 60 volume percent water and about 30 weight percent amide. Into this solution, based upon the total weight of the solution, about 1 weight percent mono-9-octadecenoate of poly (oxy-1,2-ethanediyl) sorbitol (about 20 ethanediyl groups) surfactant was added to facilitate effective dispersion of the imide agent when added to cooling water. The flask and its contents were maintained at about 80° C. with stirring until a clear solution resulted. The cooled solution was ready for use in accordance with the invention.

The relative amounts of the imide and/or salt inhibitor components required for the compositions of the invention vary depending upon the solvent medium and practicality. Thus, as the composition is diluted further and further, larger and larger amounts of the inhibitor solution must be added to the cooling water in order to achieve an effective concentration. As a practical matter, the inhibitor component must be at least 5 weight percent of the solution and is usually in the range of from about 5 weight percent to about the saturated solution value. The preferred range is from about 20 to 40 weight percent, particularly about 30 weight percent.

The inhibitors of the invention are introduced into the water of the metal-water-air contact system using usual, conventionally known procedures, as practiced in the art. Thus, the inhibitor solution or solutions are stored in an attendant storage tank and are pump-metered into the water to be treated. The initial dosage may be larger than those later metered in, that is, excess inhibitor is introduced initially. Means are provided to dynamically monitor the treatment process, including monitoring the corrosion rate of

a test sample placed in the system, chemical analysis of treated water samples, etc. Make-up water, of course, includes added inhibitor.

#### Example 3

The procedure of Example 1, *supra*, was repeated except that stannous octanoate was used in place of stannous chloride. The resulting solution was especially advantageous because in admixture with the imide solution of Example 2, *supra*, a stable solution resulted. In contrast, on standing, mixtures of the salt solution of Example 1 with the imide solutions of Example 2 clouded up and some precipitation resulted. While the solutions of Examples 1 and 2 are desirably separately added to the water to be treated, note that they need not be where shelf life of the combined components is minimal. The stannous organic carboxylate salt-imide solutions of Example 3 always require but a single inlet, irrespective of shelf life of the solution, and provide corrosion inhibition at least as effective as separate additions of the salt and imide solutions of Examples 1 and 2.

#### Corrosion Test Conditions

Corrosion tests were made using 1"×2"×1/8" carbon steel test coupons which were immersed and suspended in filtered brackish water (see Table 1 for analysis thereof) constrained in 1-liter glass flasks. The flasks were fitted with reflux condensers as well as means for bubbling air (at a rate of about 1.5 cubic feet per hour) through the flasks and contents thereof. A constant temperature of 65° C. was maintained by immersing the flasks in a constant temperature water bath.

The tests were of seven (7) days duration. The results are listed in Table 2.

TABLE 1

| Analysis       | Brackish Make-Up, PPM<br>Unless Otherwise Noted | Tower, PPM Unless<br>Otherwise Noted |
|----------------|-------------------------------------------------|--------------------------------------|
| pH             | 9.2                                             | 9.4                                  |
| Conductivity   | 17,200                                          | 35,000                               |
| TDS, MG/L      | 3,650                                           | 18,340                               |
| TSS, MG/L      | 2.4                                             | 5                                    |
| Organic Total  | 15                                              | 31                                   |
| Nitrogen       | 0.01                                            | 0.01                                 |
| Nitrate        | 5                                               | 18                                   |
| Chloride       | 13,000                                          | 64,000                               |
| Carbonate      | 94                                              | 182                                  |
| Bicarbonate    | 480                                             | 860                                  |
| Sulfate        | 1,310                                           | 2,700                                |
| Phosphate      | 2.8                                             | 8                                    |
| Sodium         | 5,710                                           | 13,000                               |
| Calcium        | 12                                              | 25                                   |
| Magnesium      | 3                                               | 5.2                                  |
| Iron           | 0.6                                             | 1.3                                  |
| Silicon        | 73                                              | 170                                  |
| Potassium      | 41                                              | 92                                   |
| Barium         | 0.3                                             | 0.6                                  |
| "P" Alkalinity | 355                                             | 844                                  |
| "M" Alkalinity | 1,660                                           | 3,400                                |

Note:

"P" Alkalinity: The alkalinity above a pH of about 8.2

"M" Alkalinity: The alkalinity between a pH of 4.3 and 8.2

TDS: Total Dissolved Solids

TSS: Total Suspended Solids

TABLE 2

| Test Results |                         |           |                              |
|--------------|-------------------------|-----------|------------------------------|
| Test No.     | Inhibitor (25 ppm)      | Rate, mpy | Corrosion                    |
| 1            | SnCl <sub>2</sub>       | 0.86      | Small pin pt. oxidation      |
| 2            | A                       | 8.17      | Wet oxidation, filiform      |
| 3            | SnCl <sub>2</sub> & A   | 2.48      | Small area of oxidation      |
| 4            | N-Octenyl Succinic Acid | 26.34     | Lots of oxidation, filiform  |
| 5            | B                       | 0.20      | One tiny spot @ hanger point |
| 6            | C                       | 0.30      | One tiny spot @ hanger point |
| 7-10         | B + C                   | 0.07      | No visible corrosion         |
| 11           | Molybdate type          | 18.20     | Severe wet oxidation         |
| 12           | Zinc & Phosphate Type   | 18.3      | Severe wet oxidation         |
| 13           | Zinc & Phosphonate Type | 8.7       | Wet oxidation                |
| 14           | None                    | 45.1      | Severe metal wastage         |

Note:

- A: N-Octenyl succinimide of allyl amine  
 B: SnCl<sub>2</sub> + sorbitol surfactant as in Example 1  
 C: N-Octenyl succinimide as in Example 2

The data of Table 2, supra, demonstrate that individually the stannous chloride and succinimide compositions herein are effective corrosion inhibitors for corrodible ferrous metal. It further demonstrates that the compositions of the invention acting in consort provide a corrosion system which is markedly superior to corrosion systems known and used in the prior art. These data further establish that the method of the invention provides effective protection for corrodible ferrous metals subject to the corrosive effects of water and air, especially brackish water and air.

The foregoing is considered as illustrative only of the principles of the invention. Further, numerous modifications and changes can readily occur. For example, while the invention has been described in connection with corrosion protection of corrodible ferrous metal, other types of metals, such as copper and aluminum, can also be protected by the principles of the invention. Therefore, it is to be understood that within the scope of the appended claims, the invention may be practiced other than as specifically described.

#### Example 4

A corrosion inhibitor blend was prepared by stirring a mixture of isopropanol and stannous octanoate with tolyltriazole and polyoxyethylated monooleate sorbitol as follows:

| Chemical                             | Percent by Weight |
|--------------------------------------|-------------------|
| Stannous Octanoate                   | 25                |
| Tolytriazole                         | 25                |
| Polyoxyethylated Monooleate Sorbitol | 3                 |
| Isopropanol                          | 47                |

These chemical concentrations can vary within a given inhibitor blend as follows: for stannous octanoate, from about 5 percent by weight to 50 percent by weight; for tolyltriazole, from about 3 percent by weight to 30 percent by weight; for polyoxyethylated monooleate sorbitol, from about 0.5 percent by weight to about 5 percent by weight; for isopropanol, 15 percent by weight to about 91.5 percent by weight. The tolyltriazole aids in providing at least two effects of an unobvious nature as a constituent of the solvent medium of the invention: inhibiting corrosion of copper

within the cooling water system as well as controlling solubility, so that the invention, when added to the cooling water, has substantial solubility and dispersability.

#### Example 5

A blend of tolyltriazole, stannous octanoate, n-alkenyl succinic anhydride, and polyoxyethylated monooleate sorbitol in 2-butoxyethanol was prepared as an industrial cooling water corrosion inhibitor. The concentrations were as follows:

| Chemical                             | Percent by Weight |
|--------------------------------------|-------------------|
| Tolytriazole                         | 20                |
| n-Alkenyl Succinic Anhydride         | 10                |
| Stannous Octanoate                   | 12                |
| Polyoxyethylated Monooleate Sorbitol | 3                 |
| 2-Butoxyethanol                      | 55                |

Variation in the above concentrations can be as follows: tolyltriazole can vary from 3 percent by weight to about 25 percent by weight; n-alkenyl succinic anhydride from 5 percent by weight to about 20 percent by weight; stannous octanoate from 5 percent by weight to 20 percent by weight; polyoxyethylated monooleate sorbitol from 0.3 percent by weight to 5 percent by weight; and 2-butoxyethanol from 30 percent by weight to about 86.5 percent by weight. Note that the tolyltriazole and n-alkenyl succinic anhydride are not reacted together but are blended along with the 2-butoxyethanol to form an improved solvent medium of the composition of the invention.

In addition to the improved characteristics noted with regard to Example 4 due to the two first-listed constituents, the solvent medium of Example 5 also has improved flash point characteristics due to the last-listed constituent, which permits usage of the invention in and about plant locations where fire ignition is a hazard.

#### Example 6

This blend was prepared and used in concert with the blends of Examples 4 and 5, above. It is composed of 1-hydroxyethylidene-1,1-diphosphonic acid treated with potassium hydroxide to a pH of 12 and carboxylate/sulfonate/nonionic functional terpolymer (tradename: "ACUMER 3100", Rohm and Haas) treated with potassium hydroxide to a pH of 8. The blend was then dissolved in water as follows:

| Chemical                                  | Percent by Weight |
|-------------------------------------------|-------------------|
| 1-hydroxyethylidene-1,1-diphosphonic acid | 15                |
| Acumer 3100                               | 15                |
| Distilled water                           | 70                |

Variation in concentration can be as follows: for 1-hydroxyethylidene-1,1-diphosphonic acid, from 5 percent by weight to 30 percent by weight; for Acumer 3100, from 3 percent by weight to about 50 percent by weight; and for distilled water, from 20 percent by weight to about 92 percent by weight. This blend also has several unobvious effects as a component of the solvent medium of the invention; inter alia, it conditions the cooling water by increasing dispersability and inhibiting scale formation. While this

blend can be added to Examples 4 and 5 before they later are dispersed in the cooling water, the preferred mode is to first add the blend of Example 6 to the cooling water followed by the addition of Example 4 or 5. The results in Table 3 were derived using the last-mentioned technique.

TABLE 3

| Corrosion Test |                       |          |              |
|----------------|-----------------------|----------|--------------|
| Test           | Corrosion             |          |              |
| No.            | Inhibitor             | Rate mpy | Surface      |
| 15             | Example 4 + Example 6 | 0.000    | No corrosion |
| 16             | Example 5 + Example 6 | 0.000    | No corrosion |

Note: For test 15 and 16, the concentration of Examples 4-6 was 25 ppm.

## Example 7

A corrosion inhibitor blend of 9 grams octenyl succinic anhydride and 12 grams stannous chloride, forming an active mixture of about 30% by weight, was combined with a suitable solvent selected from water, isopropanol, ethanol and/or propylene glycol, and then tested. Variations in solvent concentration were as discussed hereinbefore. The corrosion test condition were as set forth, supra, and resulted in a corrosion rate of about 0.02 mpy normalized to 7-day time period.

## Example 8

A corrosion inhibitor blend of 4 grams octenyl succinic anhydride, 6 grams tetraethylene pentamine and 6 grams stannous chloride, forming an active mixture of about 30% by weight, was combined with a suitable solvent selected from water, isopropanol, ethanol and/or propylene glycol, and then tested. Variations in solvent concentration were as discussed hereinbefore. The corrosion test conditions were as set forth, supra, and resulted in a corrosion rate of about 0.7 mpy normalized to 7-day time period.

## Example 9

A corrosion inhibitor blend of 5 grams octenyl succinic anhydride, 9.6 grams of tetraethylene pentamine and 6.3 grams stannous octanoate, forming an active mixture of about 30% by weight, was combined with a suitable solvent selected from water, isopropanol, ethanol and/or propylene glycol, and then tested. Variations in solvent concentration were as discussed hereinbefore. The corrosion test conditions were as set forth, supra, and resulted in a corrosion rate of about 0.01 mpy normalized to 7-day time period.

## Example 10

A corrosion inhibitor blend of 11 grams octenyl succinic anhydride, 5 grams aminoethyl piperazine, 21 grams calcium dodecyl benzene sulfonate, and 2 grams sodium dodecyl benzene sulfonate forming an active mixture of about 30% by weight, was combined with a suitable solvent selected from water, isopropanol, ethanol and/or propylene glycol, and then tested. Variations in solvent concentrated were as discussed hereinbefore. The corrosion test conditions were as set forth, supra, and resulted in a corrosion rate of about 0.9 mpy normalized to 7-day time period.

## Example 11

A corrosion inhibitor blend of 11 grams octenyl succinic anhydride, 5 grams aminoethyl piperazine, 21 grams calcium dodecyl benzene sulfonate, 2 grams sodium dodecyl benzene sulfonate and 10 grams tolyltriazole, forming an

active mixture of about 30% by weight, was combined with a suitable solvent selected from water, isopropanol, ethanol and/or propylene glycol, and then tested. Variations in solvent concentration were as discussed hereinbefore. The corrosion test conditions were as set forth, supra, and resulted in a corrosion rate of about 0.4 mpy normalized to 7-day time period.

## Example 12

10 A corrosion inhibitor blend of 13 grams n-octylamine and 9.8 grams of maleic anhydride, forming an active mixture of about 30% by weight, was combined with a suitable solvent selected from water, isopropanol, ethanol and/or propylene glycol, and tested. Variations in solvent concentration were as discussed hereinbefore. The corrosion test conditions were as set forth, supra, and resulted in a corrosion rate of about 1.5 mpy normalized to 7-day time period.

20 As to the blends set forth in Examples 10 and 11, while organic and inorganic dodecyl benzene sulfonates are set forth in detail, variations therefrom are also possible. For example, other inorganic dodecyl benzene sulfonates, such as lithium, potassium-, barium-, magnesium-, manganese-, strontium- and zinc-dodecyl benzene sulfonates, can be used. Also organic dodecyl benzene sulfonates could be utilized, such as ammonium dodecyl benzene sulfonates, and sulfonates related to polyethylene polyamines and cyclic amines, such as aminoethyl piperazine dodecyl benzene sulfonate.

## Example 13

30 A corrosion inhibitor blend was prepared by stirring stannous chloride in a solution of propylene glycol and deionized water, the amounts thereof being as follows:

| Chemical          | Percent by Weight |
|-------------------|-------------------|
| Stannous chloride | 12                |
| Propylene Glycol  | 60                |
| Deionized water   | 28                |

40 Variation in chemical concentrations normalized to a given corrosion inhibitor blend is as follows:

| Chemical          | Variation in Percent by Weight |
|-------------------|--------------------------------|
| Stannous chloride | 5 to 20                        |
| Propylene Glycol  | 35 to 80                       |
| Deionized water   | 15 to 45                       |

| Corrosion Tests Re Example 13              |                                              |          |             |
|--------------------------------------------|----------------------------------------------|----------|-------------|
| Test Specimen                              | Medium                                       | Duration | Blend Conc. |
| 1. Rectangular lead<br>(1" x 2" x 1/8")    | Potable water<br>120° F.                     | 168 hrs. | 25 ppm      |
| 2. Rectangular steel<br>(1" x 2" x 1/16")  | Plant water,<br>120° F.                      | 168 hrs. | 25 ppm      |
| 3. Rectangular copper<br>(1" x 2" x 1/16") | Plant water,<br>120° F.                      | 168 hrs  | 25 ppm      |
| 4. Rectangular steel<br>(1" x 2" x 1/16")  | Brine, 150° F.,<br>23% wt. CaCl <sub>2</sub> | 168 hrs  | 25 ppm      |

65 For the test specimens 1-4, above, a conventional test system was maintained via an air flow rate of about 1.5 cubic feet per minute. The test specimens were recovered and provided the following results.

| Test Speciment # | Corrosion Rate mpy | Surface Attack |
|------------------|--------------------|----------------|
| 1                | .00                | None           |
| 2                | .00                | None           |
| 3                | .00                | None           |
| 4                | 1.1                | Smooth         |

Furthermore, with regard to test specimen #4, the corrosion rate and occurrence of surface attack was normalized to a similar specimen where no inhibitor blend was used. A corrosion rate of 28.2 mpy was obtained. Visually, its surface was generally rough.

I claim:

1. A composition consisting essentially of (i) a stannous salt having a solubility in water of at least 0.1 percent, and (ii) a solvent medium, said stannous salt being in a range of about 5 to about 20 percent by weight, said solvent medium

having a lower alkanol content in a range of from about 35 to 80 percent by weight and a water content in a range of about 15 to about 45 percent by weight, said composition in an amount of at least 0.1 parts per million normalized to 5 water in a system that also includes air and a corrodible metal, substantially and cooperatively inhibiting corrosion of said corrodible metal.

2. The composition of claim 1 in which said stannous salt is stannous chloride.

3. The composition of claim 1 in which said lower alkanol content of said solvent medium is propylene glycol and said water content is de-ionized water.

4. The composition of claim 1 in which said stannous salt is in a range of about 12 percent by weight, and said solvent medium having an alkanol content of about 60 percent by weight and a water content of about 28 percent by weight.

\* \* \* \* \*